

June 29, 1965

P. D. JOHNSON

3,191,406

PHOTOFLASH LAMP

Filed Dec. 26, 1961



Inventor:  
Peter D. Johnson,  
by John F. Ahern  
his Attorney.

1

3,191,406  
PHOTOFLOSS LAMPPeter D. Johnson, Schenectady, N.Y., assignor to General Electric Company, a corporation of New York  
Filed Dec. 26, 1961, Ser. No. 161,803  
5 3 Claims. (Cl. 67—31)

The present invention relates to photoflash lamps in general. More particularly, the invention relates to photoflash lamps having increased burning temperature and consequent higher efficiency of chemical energy into light, higher color temperature and higher brightness.

Photoflash lamps presently utilized in photographic and allied arts generally are either of the primer type as disclosed and claimed in U.S. Patent 2,291,983—15 Pipkin or of the wire or foil type as disclosed and claimed in U.S. Patent 1,776,637—Ostermeier. In the former type photoflash lamp actinic light is produced solely by the burning of a solid combustible mixture coated upon the lamp electrode or filament, while in the latter type actinic light is produced primarily by the burning of a combustible material which may be metallic wire, shredded foil or crumpled foil distributed throughout the lamp envelope. Other forms of lamps may be utilized which include a combination or some modification of these two basic type lamps. Actinic light is generally defined as light capable of inducing chemical changes, as for instance in the emulsion of a photographic plate.

It is a principal object of the present invention to provide photoflash lamps of the aforementioned types having a high efficiency of conversion of chemical energy into actinic light.

Still another object of the invention is to provide photoflash lamps having higher color temperatures and higher peak intensities.

Briefly stated, in accord with the present invention I provide improved photoflash lamps having increased energy conversion, higher color temperatures and higher brightness in which the combustible material consist essentially of thorium, preferably of high purity.

The novel features believed characteristic of the invention are set forth in the appended claims. The invention itself, however, together with further objects and advantages thereof may best be understood by reference to the following description, taken in connection with the accompanying drawing in which the sole figure is a vertical cross-sectional view, of a photoflash lamp illustrating the invention.

In the drawing, a photoflash lamp constructed in accord with the invention comprises a hermetically sealed envelope or bulb 1 of a suitable light transmitting material such as glass, having a neck portion 2 and a solid re-entrant portion 3. A suitable base 4 is secured to neck portion 2 as by cementing or other suitable means. Bulb 1 is filled with a combustion-supporting gaseous filling which may be oxygen or a suitable oxygenous or oxidizing gas, a pressure of approximately 0.2 to 2 atmospheres, but preferably approximately 1 atmosphere. Bulb 1 may be coated on its inner or outer surface, preferably on both surfaces, with a coating of a suitable light transmitting lacquer or varnish to minimize shattering and cracking of the bulb on flashing and to render the bulb substantially shatter proof.

Sealed to the re-entrant portion 3 of bulb 1 and extending thereinto from the neck portion 2 thereof are a pair of leadin wires 5. Bridging the interior ends of wires 5 is a small ignition filament 6 which may comprise a length of wire of a suitable high resistance material such as tungsten. Mounted near the inner ends of leadin wires 5 and at least partially embedding filament 6 are thin coatings 7 of a suitable primer or combustible material causing an initial ignition flash within

2

the lamp envelope upon an application of an electric potential to wires 5. The primer material comprising coatings 7 may conveniently comprise a powdered mixture of a readily combustible metal such as zirconium and an oxygen liberating substance such as potassium chlorate or potassium perchlorate bonded together by a suitable binder such as nitrocellulose. The interior of bulb 1 is filled with a flocculent metallic mass 8 of combustible actinic light producing material, which in accord with the invention, comprises thorium. This light producing material may be in the form of fine wire shredded foil or crumpled leaf foil. Combustible material 8 is composed of thorium metal having at least 95% purity which has been protected from oxidation so as to be readily reactive with oxygen at the combustion temperature.

Conventional photoflash bulbs used heretofore are similar to the bulbs of my invention, but utilized, as the flocculent metallic mass of actinic light producing material, generally aluminum or magnesium. Numerous other materials have been mentioned for this type material including copper, iron, nickel, and rare earths generally. The staple materials utilized, however, generally constitute aluminum and/or magnesium.

In accord with my invention, the thorium metal is of 95% purity or better and is unoxidized. If it is in the form of a leaf foil it should be of a thickness of 0.001" or less, and is preferably shredded into fine shreds to be more readily combustible in a short period of time. In certain instances when long combustion period is desired foil or shredded foil of thickness greater than 0.001" may be used, thus facilitating a longer burning time. In bulbs of the invention light is actually emitted by excited thorium oxide produced by the reaction of thorium with the atmosphere in the bulb.

The atmosphere within bulb 1 generally comprises oxygen. When mixtures of oxygen and nitrogen are used nitrogen may react with thorium and contribute to the light output. The amount of oxygen and of thorium in the bulb depends upon the size and volume of the bulb. In one embodiment, a 7 cubic centimeter approximate volume bulb utilizes approximately 60 milligrams of shredded foil thorium and an oxygen pressure of 1000 millimeters of mercury. In another embodiment a 25 cubic centimeter approximate volume bulb was utilized and contained 150 milligrams of thorium and utilized oxygen at a pressure of 700 millimeters of mercury.

In general, the ratio of thorium to oxygen within the bulb varies within the range of from 5 to 25 milligrams of thorium per cubic centimeter of oxygen at atmospheric pressure.

The criteria of measurement of a material as an actinic light source in a photoflash lamp are the color temperature, the peak intensity and the efficiency of conversion of chemical energy into light energy. Color temperature generally refers to the absolute temperature in degrees Kelvin of a theoretical black body radiator whose color appearance matches that of the light source being measured. For conventional photoflash lamps utilizing aluminum as the actinic light source and which are generally utilized commercially today, the average color temperature is approximately 3800° K. Lamps constructed in accord with this invention, although not in mass production to the extent that an average color temperature can be reached with exact precision, generally show an average color temperature of the order of 4500° K., with some measurements going as high as 5000° K. Accordingly, in the measurement of color temperature photoflash lamps constructed of high purity unoxidized thorium are highly advantageous and superior to present day commercial photoflash lamps.

Another criteria of photoflash lamps is the peak intensity of the light emitted by the lamp. This is dependent on

the temperature of the radiating material and, according to Planck's Radiation Law, increases rapidly with increase in temperature. Calculations made from the thorium lamps which have been constructed in accord with the present invention indicate a maximum peak intensity of these lamps which is approximately 4 to 6 times greater than the average peak intensity of aluminum filled photoflash lamps. Finally, the efficiency of conversion of chemical energy into light energy is approximately 20% for lamp constructed in accord with the present invention as compared with 10% for conventional aluminum filled photoflash lamp.

One specific example, given for illustrative purposes only and not to be construed in a limiting sense, of a preferred embodiment of the invention comprises the lamp as illustrated in the drawing and having an elliptical glass envelope with a major axis of 1.58" and a minor axis of 1.38". The bulb has a volume of approximately 25 cubic centimeters and is filled with 0.001" thick unoxidized thorium metal having a purity of approximately 98% shredded into filaments of approximately 0.001" width and amounting to a total weight of approximately 175 milligrams of thorium metal. The remainder of the bulb is filled with oxygen gas at a pressure of approximately 1 atmosphere. The primer coating on the load wires is approximately  $\frac{1}{6}$ " long and approximately 0.003" thick. The filament is a 0.0007" diameter tungsten wire.

In accord with another embodiment of the present invention, the thorium actinic light producing material may be included in the primer beads 7 which are, consequently made much greater in weight, and the shredded foil 8 is thereby eliminated from the envelope. As with the embodiment illustrated in the drawing wherein beads 7 merely comprise a starter the combustible material, thorium replaces the zirconium and is in the form of a finely divided powder having a purity of 95% or better and unoxidized. One specific example of a bulb constructed with in accord with this embodiment was a bulb, as in the first example, having a volume of approximately 25 cubic centimeters in which the total combustible mixture of both beads 7 comprise approximately 30 milligram thorium powder and 40 milligram potassium perchlorate. The bulb was also filled with oxygen to a pressure of approximately 300 millimeters of mercury. Alternatively, ammonium perchlorate could be utilized instead of the potassium perchlorate.

The photoflash lamps of this invention may be produced in accord with the standard manufacturing techniques. The lamp illustrated in the drawing utilizing a wire of foil type actinic light producing combustible material may be produced in accord with the teachings of U.S. Patent 2,351,290—Rippl et al. Likewise, the bulbs of the second described embodiment wherein the combustible material comprises only beads 7 may be produced in accord with the aforementioned patent 2,291,983—Pipkin.

While I have described the invention with reference to certain embodiments thereof many modifications will occur to those skilled in the art. Accordingly, I intend by the appended claim to cover all such modifications as come within the true spirit and scope of the invention.

What I claim as new and desire to secure by Letters Patent of the United States is:

1. A photoflash lamp comprising an hermetically sealed light transmitting envelope; an oxygenous atmosphere within said envelope; and a charge of a combustible material within said envelope sufficient, on combustion within said envelope, to produce actinic light of a brightness corresponding to that of a black body radiator at the combustion temperature of thorium, said material comprising unoxidized thorium metal having purity of at least 95%.

2. A photoflash lamp comprising an hermetically sealed light transmitting envelope; an atmosphere of oxygen within said envelope, and a charge of a combustible actinic light producing material within said envelope sufficient, on combustion within said envelope, to produce actinic light of a brightness corresponding to that of a black body radiator at the combustion temperature of thorium, said material comprising unoxidized thorium.

3. A photoflash lamp comprising an hermetically sealed light transmitting envelope; an atmosphere of oxygen within said envelope, and a charge of a combustible actinic light producing material within said envelope sufficient, on combustion within said envelope, to produce actinic light of a brightness corresponding to that of a black body radiator at the combustion temperature of thorium, said material comprising unoxidized thorium; said thorium and said oxygen being present in proportions of 5 to 25 mg. of thorium per cubic centimeter of oxygen at atmospheric pressure.

#### References Cited by the Examiner

#### UNITED STATES PATENTS

|           |       |                 |       |        |
|-----------|-------|-----------------|-------|--------|
| 594,594   | 11/97 | Bostwick        | ----- | 149—19 |
| 613,021   | 10/98 | Schwartz        | ----- | 149—9  |
| 1,776,637 | 9/30  | Ostermeier      | ----- | 67—31  |
| 2,012,866 | 8/35  | Decker          | ----- | 149—42 |
| 2,071,369 | 2/37  | Williams et al. | ----- | 67—31  |
| 2,272,779 | 2/42  | Sarbey          | ----- | 67—31  |
| 2,813,412 | 11/57 | Johnson         | ----- | 67—31  |

#### FOREIGN PATENTS

14,972 10/06 Great Britain.

#### OTHER REFERENCES

Metal Progress: "Non-Nuclear Uses of Thorium," by W. C. Lilliendahl, February 1957, pp. 104—107, vol. 71, No. 2, pub. by American Society for Metals, Mount Morris, Ill.

EDWARD J. MICHAEL, Primary Examiner.

PERCY L. PATRICK, Examiner.